

2,901,317

## ANTI-CAKING AGENT FOR AMMONIUM NITRATE

Paul O. Marti, Jr., Munster, Ind., assignor to Standard Oil Company, Chicago, Ill., a corporation of Indiana

No Drawing, Application December 31, 1952  
Serial No. 329,146

11 Claims. (Cl. 23—103)

This invention relates to a particulate ammonium nitrate composition which is substantially non-caking and substantially free-flowing at atmospheric humidity. Also, the invention relates to an improved method of grinding ammonium nitrate in the presence of atmospheric humidity.

Ammonium nitrate is hygroscopic. In the presence of atmospheric humidity particulate ammonium nitrate takes up moisture and the individual particles tend to agglomerate to form lumps; under conditions of high humidity the ammonium nitrate particles tend to form a solid mass. This agglomeration tendency of ammonium nitrate in the presence of atmospheric humidity is commonly called "caking" or "setting."

For most commercial uses it is desirable that the ammonium nitrate particles be free-flowing, e.g., when used as fertilizer, it is necessary that the granules flow readily from the hopper through the distributing slots onto the ground. For use in the explosive industry the powdered ammonium nitrate should flow readily from the storage bins into the mixing vessel. Bagged ammonium nitrate granules tend to cake and this cake must be broken up before use.

Unless considerable care is taken to maintain low atmospheric humidity, it is extremely difficult to obtain powdered ammonium nitrate of a particle size suitable for explosive use. Even with care regarding atmospheric humidity, it is at present a slow and expensive grinding operation to prepare finely powdered ammonium nitrate.

It is an object of this invention to prepare a particulate ammonium nitrate composition that is not susceptible to atmospheric humidity. Another object of the invention is a composition consisting of ammonium nitrate particles coated with a defined anticaking-agent. Still another object is a composition consisting of ammonium nitrate particles coated with a comminuted agent, which composition is characterized by essentially free-flowability at atmospheric humidity and by a storage stability substantially that of dynamite grade ammonium nitrate. A particular object of the invention is a method of grinding ammonium nitrate in the presence of atmospheric humidity to produce powdered ammonium nitrate more quickly and more cheaply than by the prior art methods. Another particular object is an improved method of grinding ammonium nitrate in the presence of atmospheric humidity which consists of grinding ammonium nitrate particles in the presence of a defined anticaking-agent (grinding aid).

It has been discovered that ammonium nitrate particles coated with comminuted copper oxide are substantially non-caking in the presence of atmospheric humidity.

The improved method of grinding ammonium nitrate in the presence of atmospheric humidity grinds ammonium nitrate particles in the presence of an effective amount of said comminuted agent; preferably using an amount at least sufficient to substantially coat the surface of the ammonium nitrate particles produced in the grinding operation.

The term "ammonium nitrate" as used in this specification and in the claims is intended to include either ordinary commercial grade ammonium nitrate or dynamite grade ammonium nitrate or pure ammonium nitrate.

5 The term "atmospheric humidity" is intended to mean the presence of water vapor in air at various temperatures; or even the atmospheric condition commonly known as fog. More particularly, the term is intended to include those conditions at which the water vapor present in the 10 air would cause agglomeration and caking of ammonium nitrate particles.

The copper oxide anticaking-agents of this invention may be either anhydrous or may contain small amounts of adsorbed water. Either the naturally occurring material or synthetic material may be used. The preferred individual members are: Cupric oxide, CuO; cuprous oxide, Cu<sub>2</sub>O.

15 The anticaking-agents (grinding aids) of this invention must have a particle size markedly smaller than the 20 particle size of the ammonium nitrate which is to be treated. In order to obtain substantially complete coating a comminuted mixture of the agent is preferred. Especially effective agents have a particle size between about 0.01 and about 10 microns; as much as 10 weight 25 percent of particles having an average size somewhat greater than 10 microns may also be present. It is preferred to use agents having a particle size mainly below about 1 micron when the agent is intended for use solely as an anticaking-agent.

30 The anticaking-agent appears to operate by forming an adherent coating on the outer surface of the ammonium nitrate particle. This coating of agent substantially precludes the water vapor in the atmosphere from contacting the ammonium nitrate. Furthermore, the agent particles 35 reduce the agglomerating tendencies of the ammonium nitrate particles so that the flow characteristics of the particulate coated-ammonium nitrate is better than that of the uncoated particles even in a dry atmosphere. The coating slows, somewhat, the rate of solution of the nitrate in liquid water; however, the solubility in liquid water is not changed.

40 The anticaking-agents of this invention adhere readily to the ammonium nitrate particles. A non-caking composition is easily obtained by simple mixing of ammonium 45 nitrate particles and a suitable amount of the anticaking-agent. More finely divided coated ammonium nitrate particles may be obtained by passing simultaneously ammonium nitrate particles and a suitable amount of anticaking-agent through a grinder. The improved grinding 50 operation can be carried out by first mingling the ammonium nitrate particles and the comminuted anticaking-agent and then grinding the mingled materials; or the ammonium nitrate particles and the anticaking-agent may be added simultaneously as separate streams into the 55 feed chamber of the grinder. When operating with minimum amounts of anticaking-agent (grinding aid), it may be desirable to regrind the product from the first grinding operation.

Some improvement in caking characteristics can be obtained by the addition of small amounts of agent. For best results and maximum improvement in caking characteristics at least sufficient agent should be added to the ammonium nitrate particles to substantially coat the entire outer surface of the ammonium nitrate particles.

60 Amounts of agent in excess of this quantity have no significant beneficial effect on the free-flowability of the coated ammonium nitrate particles. The amount of anticaking-agent needed to coat a given quantity of ammonium nitrate particles is dependent upon the size of the 65 ammonium nitrate particles. The smaller the particles the more agent needed per unit weight of ammonium nitrate. For fertilizer size grains as little as 0.2 weight 70 ammonium nitrate particles.

percent, based on ammonium nitrate, of cupric oxide or cuprous oxide is sufficient. For the ammonium nitrate particles in so-called dynamite grade, between about 0.5 and 1.0 weight percent of cupric oxide or cuprous oxide may be needed. For the fine powder desirable for some explosive usages wherein most of the particles pass through a 325 mesh screen as much as 4 or 5 weight percent of cupric oxide or cuprous oxide may be needed. In general the amount of anticaking-agent needed to obtain a particulate ammonium nitrate composition characterized by essentially free-flowability at atmospheric humidity is between about 0.2 and 5 weight percent of comminuted anticaking-agent wherein the larger amount corresponds to the finer average particle size of the ammonium nitrate.

The anticaking-agents of this invention catalyze the decomposition of ammonium nitrate. The presence of copper oxide in ammonium nitrate can result in an explosion when the ammonium nitrate is heated to about 130° C. The higher the purity of the ammonium nitrate, the more catalyst required. The presence of copper oxide markedly increases the rate of decomposition, as measured by gas evolution, at higher atmospheric temperatures. However, in general, the amounts of anticaking-agents needed to produce free-flowing ammonium nitrate particles at atmospheric humidity are sufficiently less than the amounts needed to catalyze the decomposition of ammonium nitrate that the coated particles are characterized by storage stability substantially that of dynamite grade ammonium nitrate. Dynamite grade ammonium nitrate contains a sufficient amount of impurities such that the stability is not as great as pure ammonium nitrate; nevertheless, the stability of the dynamite grade is sufficient for all explosive purposes.

In order to illustrate the results obtainable with the anticaking-agents of this invention, the following illustrative examples are set forth:

#### Example I

Run 1.—This was carried out with Hercules dynamite grade ammonium nitrate. This material was analyzed for particle size distribution using the Rotap screen analysis method. The analysis was carried out at a room temperature of about 70° F. and a relative humidity of about 30%. The analysis showed the following particle size distribution:

| Screen mesh number: | Wt. percent retained |
|---------------------|----------------------|
| +10                 | 0.2                  |
| +14                 | 2.6                  |
| +30                 | 80.0                 |
| +80                 | 12.5                 |
| -80                 | 4.7                  |

A quantity of this ammonium nitrate was placed in an 8-ounce screw-top jar. The top was loosely screwed on so that the atmosphere would have access to the interior of the jar. The jar was placed on a shelf in a room; after 7 days' exposure to room temperatures between about 70 and 85° F. and relative humidities of between about 30 and 70%, the ammonium nitrate particles had caked not only together, but had adhered to the glass surface. It was possible to invert the jar without any of the ammonium nitrate particles becoming detached from the mass or the mass becoming detached from the bottom of the jar.

Run 2.—This was carried out by mixing about 1 weight percent of commercial grade cupric oxide, based on ammonium nitrate, with the same amount of ammonium nitrate particles as used in run 1. The mixing was accomplished by stirring the oxide and the ammonium nitrate particles with a spatula.

An electron microscopic examination of the oxide showed that the particle size ranged from 0.01 to about 10 microns; most of the particles were less than 1 micron in size.

Microscopic examination of the mixture showed that the ammonium nitrate particles were completely coated with a layer of oxide. The individual particles were of the same color as the oxide.

The coated particles were stored in a loosely screw-capped bottle. The particles flowed quite easily and contained no lumps after 2 months' exposure to room temperatures of between 70 and 85° F. and relative humidities between about 20 and 80%.

Run 3.—A test was made with cuprous oxide under the same conditions as run 2. The results with the cuprous oxide appeared to be identical with those of the cupric oxide.

#### Example II

Run 4.—Dynamite grade ammonium nitrate was ground in a Mikro-Pulverizer at a speed of 9600 r.p.m. using a slotted screen at a relative humidity of 70%. The first ground material was reground under the same conditions to maximize the finer particles. The Rotap screen analysis of this material was:

| Screen mesh number: | Wt. percent retained |
|---------------------|----------------------|
| +80                 | 0.3                  |
| +120                | 4.7                  |
| +200                | 37.0                 |
| +325                | 35.0                 |
| -325                | 23.0                 |

A quantity of this 9600 r.p.m. material was placed in an 8-ounce glass jar as described in run 1. After 2 days' exposure to room temperature of about 75° F. and a relative humidity between about 50 and 70%, the material was caked solid and adhered firmly to the glass jar. The jar could be inverted without detaching any of the caked material.

Run 5.—About 3 weight percent of cupric oxide (same as in run 2) was added to a quantity of the 9600 r.p.m. material. Microscopic examination of the mixture showed the ammonium nitrate particles to be completely coated with a layer of the agent. After 2 months' exposure to the same atmospheric conditions as those given in run 2 the coated ammonium nitrate was still substantially free-flowing, although some very small lumps had formed.

Run 6.—This run used cuprous oxide as the agent. Under the conditions of run 5, it appears that cuprous oxide and cupric oxide are equally effective as anticaking-agents.

#### Example III

Run 7.—Dynamite grade ammonium nitrate was ground in the Mikro-Pulverizer at 9600 r.p.m. The ground material was ground a second time. The room temperature during the grinding was about 75° F. and the relative humidity was about 90%. The ground material tended to "blind" the screen. The total grinding time for 200 grams of ammonium nitrate charged was somewhat more than one-half hour.

The 9600 r.p.m. material formed lumps in a short time and in about 2 days was caked solid when exposed in a loosely capped jar to a room temperature of about 75° F. and a relative humidity of about 70-80%.

The Rotap screen analysis of this 9600 r.p.m. material—made immediately after grinding—was:

| Screen mesh number: | Wt. percent retained |
|---------------------|----------------------|
| +80                 | 8                    |
| +150                | 22                   |
| +200                | 17                   |
| +325                | 23                   |
| -325                | 30                   |

Run 8.—Under the same atmospheric conditions as those given in run 6, 200 grams of dynamite grade ammonium nitrate and 6 grams of cupric oxide were charged to the Mikro-Pulverizer operating at 9600 r.p.m. The ammonium nitrate and the oxide were commingled by

shaking in a jar before being charged to the hopper. The total time for two passes through the pulverizer in this run was about 5 minutes. The Rotap analysis of the coated ammonium nitrate product from this run was:

| Screen mesh number: | Wt. percent retained |
|---------------------|----------------------|
| +80                 | 1                    |
| +150                | 13                   |
| +200                | 18                   |
| +325                | 22                   |
| -325                | 46                   |

This run illustrates the remarkable reduction in grinding time obtained by the use of comminuted copper oxide as a grinding aid and the simultaneous considerable decrease in average particle size of the product ammonium nitrate. It is obvious that a considerable decrease in speed of the Mikro-Pulverizer can be made when using grinding aid in order to obtain the same particle size distribution as that given in run 6.

Electron microscopic examination of the product ammonium nitrate particles showed the ammonium nitrate to be substantially completely coated with a layer of oxide. The coated ammonium nitrate particles showed only a few very small lumps after about 2 months' exposure to the conditions of run 2.

Thus having described the invention, what is claimed is:

1. A particulate composition consisting of ammonium nitrate particles coated with a comminuted copper oxide, which coated particles are characterized by substantially free-flowability at atmospheric humidity and by a storage stability substantially that of dynamite grade ammonium nitrate.

2. The coated particles of claim 1 wherein said oxide is cupric oxide.

3. The coated particles of claim 1 wherein said oxide is cuprous oxide.

4. A particulate composition consisting of ammonium nitrate particles coated with between about 0.2 and 5 weight percent, based on ammonium nitrate, of a copper oxide, having a particle size between about 0.01 and 10 microns, where the smaller percentage corresponds to larger ammonium nitrate particles, and which composition

is characterized by free-flowability at atmospheric humidity and by a storage stability substantially that of dynamite grade ammonium nitrate.

5. The composition of claim 4 wherein said oxide is selected from the class consisting of cupric oxide and cuprous oxide.

6. An improved method of grinding ammonium nitrate in the presence of atmospheric humidity, which method consists of grinding ammonium nitrate particles in the presence of a comminuted copper oxide to obtain nitrate particles of size smaller than those charged.

7. The method of claim 6 wherein the particle size of said oxide is between about 0.01 and 10 microns.

8. The method of claim 6 wherein said oxide is cupric oxide.

9. The method of claim 6 wherein said oxide is present in an amount at least sufficient to substantially coat the surface of the product ammonium nitrate particles.

10. An improved method of grinding ammonium nitrate particles in the presence of atmospheric humidity, which method consists of grinding ammonium nitrate particles in the presence of between 0.3 and 5 weight percent, based on the nitrate, wherein the larger amount corresponds to the finger average particle size of the ammonium nitrate, of copper oxide, having a particle size between about 0.01 and 10 microns, which product nitrate particles are of a smaller size than the particles charged.

11. A non-caking ammonium nitrate composition which consists of ammonium nitrate particles having a Rotap screen analysis: +14 mesh, about 3 wt. percent; +30 mesh, about 80 wt. percent; +80 mesh, about 12 wt. percent; and -80 mesh, about 5 wt. percent; coated with about 1 wt. percent, based on nitrate, of cupric oxide, having a particle size between about 0.01 and 10 microns, mainly below about 1 micron.

#### References Cited in the file of this patent

#### UNITED STATES PATENTS

- |    |           |               |              |
|----|-----------|---------------|--------------|
| 40 | 286,132   | Harned        | Oct. 2, 1883 |
|    | 2,274,822 | Cairns et al. | Mar. 3, 1942 |